# EUROPEAN PATENT SPECIFICATION

(11) **EP 0 532 500 B1**
(45) Date of publication and mention of the grant of the patent: **10.05.1995**
(21) Application number: 91905651.5
(22) Date of filing: 28.02.1991
(51) Int. Cl.: D06M 15/693, F16L 11/10

(54) **BRAIDED PRODUCT AND METHOD OF MAKING SAME**
GEFLECHTE UND DESSEN HERSTELLUNGSVERFAHREN
PRODUIT TRESSE ET SON PROCEDE DE FABRICATION

(30) Priority: 12.03.1990 US 492802
(43) Date of publication of application: 24.03.1993
(73) Proprietor: THE BENTLEY-HARRIS MANUFACTURING CO., Lionville, Pennsylvania 19353 (US)
(72) Inventor: KITE, J., Sellers, III, Carefree Arizona AZ 85377 (US)
(74) Representative: Crux, John Anthony
(86) International application number: US9101303
(87) International publication number: WO9114034

(56) References cited:
- GB-A- 697 847
- GB-A- 1 422 936
- GB-A- 1 448 601
- US-A- 2 393 530
- US-A- 2 977 839
- US-A- 3 048 078
- US-A- 3 334 165
- US-A- 4 452 279
- US-A- 4 754 685
- US-A- 4 870 887

## Description

### Field of the Invention

This invention relates to monofilament braided product and to methods for making same. It relates more particularly to braided product made up of monofilaments, typically of a resilient engineering plastic material and typically (but not necessarily) in the form of a tubular sleeve.

### Background of the Invention

One known form of braided product is the Expando™ self-fitting protective oversleeve made by Bentley-Harris Manufacturing Co. of Lionville, Pennsylvania. This tubular sleeve is expandable in that, when the ends are pushed toward each other it expands in diameter, and when they are released it returns to its original shape and size. This enables it to be pulled or pushed over objects of different diameters, including diameters greater than the unstressed or "rest" diameter of the sleeve, and also enable it to accommodate expansion, bending and twisting of hoses or wires which may run through it. This expandable braided product also exhibits a "spring-back" or "memory" characteristic, whereby it tends to return to its rest diameter when released from longitudinal forces. Such expandable braided sleeving has been widely used, for example to protect, and/or dress, wiring harnesses and hose assemblies.

One difficulty with the typical braided product of the expandable type is that when the braid is cut in an ordinary manner, as by scissors, the ends of the braid will tend to unravel or splay, the braiding coming apart for a substantial distance from the cut ends. This is particularly troublesome when an end of a braided sleeve must be forced over a large-diameter object, causing the monofilaments to splay and therefore no longer provide the desired type of tight fit on the smaller-diameter contents of the tubular covering; in addition such splaying is cosmetically very undesirable.

There are currently three principal ways in which this problem has been addressed, as follows:
(1) Coat the braided product with a continuous coating. This eliminates the splaying, but also restricts the expandability of the braid and therefore its ability to slide over, or wrap around, an object with full conformity to a variable cross-section of the object. Such a construction also prevents one from "breaking out" a branching wire from the interior of braided tubing, as is sometimes desirable.
(2) Heat-set the braided product. Heating the completed product will put a slight set into the braid, but with even slight mechanical expansion the ends will unbraid and splay out again.
(3) Cut the braid with a hot knife or wire. With most plastic braidings, the sleeve can be cut through with a hot knife or wire, thereby fusing the monofilaments to each other to prevent the braid from fraying or unravelling. However, such end treatment will fix the diameter at that set by the fusing of the end of the tubular braid, and thereby prevent the braid from expanding readily to receive a large object. Further, this method requires use of special hot melt devices to provide such cutting of the braid, and therefore is not useful for field installations of the sleeve where no such special tools are available.

Prior art patents include US-A-3334165 which discloses an overall coating of nylon as an impermeable, essentially protective sheath on top of a braid used to reinforce a hose. GB-A-144860 discloses a method of making a continuous strip of a bias-cut woven fabric by applying a curable liquid binder to stabilise the fabric in its as-cut state, prior to use as reinforcement for a drive belt.

US-A-4870887 discloses a braided sleeve containing a rigid filament, for example a stainless steel wire, to prevent splaying of the sleeve when cut. Optionally the sleeve is coated with a polymeric material.

US-A-3048078 discloses a method of making an extensible electrical cable in which a textile braid is incorporated into an outer insulation layer of rubber.

Of the foregoing, only US-A-4870887 addresses the splaying problem mentioned earlier, but for many applications it is undesirable to incorporate a rigid filament. Accordingly, it is an object of the present invention to provide a new braided product and method of making it, which minimise such fraying whilst retaining the natural expansion and contraction characteristics of the expandable type of braided product.

It is also an object of the invention to provide such method in which the treatment providing the above described advantageous characteristics is readily and inexpensively performed, and in which the user can cut the resultant braided product to the desire length without having to use any special cutting or bonding tools.

### Summary of the Invention

These and other objects of the invention are achieved by the provision of an expandable braid comprising a plurality of braided monofilaments in which the braid is coated with an adherent solid elastomeric material extending from over-weave monofilaments to their associated underweave monofilaments at their respective cross-overs, thereby permitting the monofilaments to pivot with respect to each other as required to retain the desired expandable characteristics, while preventing splaying, the openings between said monofilaments being substantially free of said coating.

The coating is preferably applied by passing the braid continuously through a liquid bath containing the elastomeric coating material in flowable form, and then solidifying the coating in position on the braided product. The viscosity of the liquid of the coating is such that it provides enough material in the proper places to fix the monofilaments against end splaying, while retaining the ability of the filaments to pivot with respect to each other, and the consequent ability of the sleeve to expand and shrink in cross-sectional size. If the coating does initially extend across the openings between the monofilaments, it is preferably broken by longitudinal compression of the braided material.

In this manner there is provided a braided product and method of making it which prevent splaying of the end of the braid without materially adversely affecting the expandable characteristics of the braid.

### Brief Description of Figures

These and other objects of the invention will be understood from a consideration of the following detailed description taken in connection with the accompanying drawings, in which:
Figure 1 is a side view of a section of expandable tubular product which has been cut by an ordinary pair of scissors, and mechanically expanded at the cut end, and which exhibits substantial splaying at its end;
Figure 2 is a side view of a section of expandable braided product made in accordance with the invention, cut at its end with an ordinary pair of scissors and then subjected to a similar expanding procedure;
Figure 3 is an enlarged fragmentary view of the exterior of the braided product of Figure 2;
Figure 4 is a cross-sectional view taken on lines 4-4 of Figure 3, showing the braided product of the invention after the coating has been formed therein;
Figure 5 is a cross-sectional view taken along lines 5-5 of Figure 3 ; and
Figure 6 is a cross-sectional view like Figure 5, but illustrating the condition in which a break exists in the coating near each cross-over of the braid.

### Detailed Description of Specific Embodiments

Referring now to the embodiment of the invention shown in the drawings by way of example only, and without thereby limiting the scope of the invention, Figure 1 shows a section of expanded, braided tubular sleeving 8, constructed in accordance with the prior art and exhibiting undesired splaying of the monofilaments at its end 9. Figure 2 shows a length of expandable, braided, tubular sleeving 10 in accordance with the present embodiment of the invention. It is made up of monofilaments such as 11, 12, 13, 14 in a simple single-strand two-over, two-under braid pattern. Each monofilament in this example is of engineered plastic, for example nylon or polyester, and is substantially rectangular in cross-section. The monofilaments are covered with an adherent elastomeric coating 16. In some cases, particularly after expansion and contraction of the braid by pulling and pushing of its ends, the coating may contain a break where one monofilament crosses another, as indicated by the break lines such as 20, 21 in Figure 6.

In this preferred embodiment of the invention the coating does not decrease substantially the areas of the openings such as 30, 31 between the monofilaments, so that space remains for the filaments to pivot at the cross-overs, one with respect to its adjacent neighbour, during expansion and contraction of the sleeve, according to the usual characteristic of such expandable braids. The elastomeric coating tends to fix the positions of the cross-overs, but being elastomeric, it permits the necessary pivoting of the monofilaments with respect to each other. This fixing action of the elastomer material prevents the ends from splaying, as is important for the reasons pointed out above. The retention of the openings such as 30, 31 also permits a wire or the like to be extracted and passed outwardly from the sleeve if so desired.

While there may be a variety of methods by which the coating may be applied, it is preferred to accomplish it by passing a continuous sleeve of the braided material through a bath of the coating material and then drying it in an oven.

One presently-preferred example of the improved braided product and of a method for making it, is as follows:

A continuous, expandable braided tube of about 9.5mm (9.5x10⁻³ metres) rest diameter is made in conventional manner from 48 monofilaments of 11.1 tex, (100 denier) nylon, each monofilament about 0.75mm (30 mils) wide and about 0.25mm (10 mils) in thickness; the braided tubing is typically coiled on a spool in long lengths, eg, 609.6 metre lengths. The tubing from the spool is then run lengthwise downward into and through a bath of the coating material, continuing upwardly therefrom through a hot-air oven typically operating at about 150°C.

The liquid coating material may be resorcinol formaldehyde, with a viscosity of 15 N/s/m⁻², (15,000 centipoises) or less so that it will coat the monofilaments in the braid without closing the openings between them. Preferably the tubing is subjected to stretching while passing through the bath, and until drying of the coating is complete.

The resultant braided tubing can be cut to length with ordinary scissors, and will then exhibit minimal tendency toward splaying. Nevertheless, when longitudinally compresses it will increase its diameter, and it will also exhibit memory in that, when unstressed, it tends to return to the diameter and length it had before compression.

In general, the invention is applicable to a wide variety of sizes, shapes and materials of braids and of monofilaments, including monofilaments of round cross-section; it is also of wide applicability with respect to the number of monofilaments in the braid. While many important applications of the invention involve a tubular braid, the invention is also useful in making flat, mat-like expandable braid products. Also, while the coating material is preferably elastomeric, at least some of the advantages of the invention may be realised by using a non-elastomeric material for the coating which does not bond the filaments rigidly together, but instead fractures upon compression and/or stretching of the braid, leaving low walls of coating material on each side of each monofilament at each cross-over to provide a positioning channel, or at least a high-friction surface, which resists the type of displacement of the monofilaments which occurs during splaying. A similar effect exists in some case when an elastomeric material is used which fractures during stretching and/or compression. Other coating procedures may also be used, so long as they do not result in such a thick, pervasive coating that the monofilaments cannot pivot, each with respect to its neighbour, as is required to exhibit the desired expandable characteristic.

## Claims

1. An expandable braid comprising a plurality of braided monofilaments and a coating of an adherent solid elastomeric material on said filaments holding said filaments in their proper relative positions to prevent splaying of the ends of said braid while permitting them to pivot with respect to each other at each of their cross-overs so as to retain the expandable characteristics of said braid, the openings between said monofilaments being substantially free of said coating.

2. An expandable braid according to claim 1, wherein said elastomeric material is selected from the group consisting of resorcinol formaldehyde and acrylic latex.

3. An expandable braid according to claim 1, or claim 2, wherein said monofilaments are of engineered plastic material.

4. An expandable braid according to claim 3, wherein said monofilaments are of nylon or polyester.

5. An expandable braid according to any of claims 1-4, wherein said coating extends over substantially all of the exposed surfaces of said monofilaments throughout the length of said braid.

6. An expandable braid according to any preceding claim, wherein said coating is from about 0.025mm to about 0.5mm (about 1 to about 20 mils) in thickness.

7. A method of treating an expandable braid comprising a plurality of braided monofilaments to reduce its tendency to splay at its ends while retaining its expandable properties, characterised by the step of forming a solid coating of an adherent solid elastomeric material on said monofilaments of said braid to hold them in their proper relative positions and thereby minimise the tendency toward splaying at the ends of said braid, said coating permitting said monofilaments to pivot with respect to each other at their cross-overs so as to retain the expandable characteristics of said braid, said forming step comprising coating substantially all exposed surfaces of said monofilaments with said elastomeric material in flowable form without filling the openings between said monofilaments.

8. A method according to claim 7, wherein said material is selected from the group consisting of resorcinol formaldehyde and acrylic latex.

9. A method according to claim 7 or claim 8, wherein said coating is from about 0.025mm to about 0.5mm (about 1 to about 20 mils) in thickness.

10. A method according to any of claims 7 to 9, wherein said forming of said coating comprises passing said braid through a bath of the elastomeric material in its flowable form, and thereafter allowing said material to solidify on said braid.

11. A method according to claim 10, wherein said elastomeric material in its flowable form has a viscosity not substantially greater than 15 N/s/m⁻² (15,000 centipoises).

12. A method according to any of claims 7 to 11, comprising forming said solid coating over said monofilaments and the openings between them, and thereafter compressing said braided product to break open said coating in the regions where it covers said openings.

## Patentansprüche

1. Ausdehnbares Geflecht umfassend eine Mehrzahl von geflochtenen Monofilamenten und eine Beschichtung eines anhaftenden festen elastomeren Materials auf diesen Fäden, welche diese Fäden an ihren richtigen Stellungen zueinander hält, um Aufspleißen der Enden dieses Geflechts zu vermeiden, während sie sich gegeneinander an jeder ihrer Überkreuzungsstellen drehen bzw. verschwenken können, so daß die Ausdehnungsmerkmale eines solchen Geflechts erhalten bleiben, wobei die Öffnungen zwischen diesen Monofilamenten praktisch frei von dieser Beschichtung sind.

2. Ausdehnbares Geflecht nach Anspruch 1, dadurch gekennzeichnet, daß das elastomere Material aus der Gruppe gewählt ist, die aus Recorcin/Formaldehyd und Acryllatex besteht.

3. Ausdehnbares Geflecht nach Anspruch 1 oder 2, dadurch gekennzeichnet, daß die Monofilamente aus Kunststoffkonstruktionsmaterial sind.

4. Ausdehnbares Geflecht nach Anspruch 3, dadurch gekennzeichnet, daß die Monofilamente aus Nylon oder Polyester sind.

5. Ausdehnbares Geflecht nach irgendeinem der Ansprüche 1 bis 4, dadurch gekennzeichnet, daß sich die Beschichtung über praktisch die Gesamtheit der freiliegenden Oberflächen dieser Monofilamente durch die Länge dieses Geflechts erstreckt.

6. Ausdehnbares Geflecht nach irgendeinem der vorhergehenden Ansprüche, dadurch gekennzeichnet, daß die Beschichtung etwa 0,025 mm bis etwa 0,5 mm (etwa 1 bis etwa 20 mils) Dicke hat.

7. Verfahren zur Behandlung eines ausdehnbaren Geflechtes, umfassend eine Mehrzahl von verflochtenen Monofilamenten, zur Verminderung seiner Neigung an den Enden aufzuspleißen, während seine Ausdehnungseigenschaften beibehalten bleiben, gekennzeichnet durch die Stufe der Bildung einer festen Beschichtung eines anhaftenden festen elastomeren Materials auf diesen Monofilamenten dieses Geflechts, um sie in ihren richtigen relativen Stellungen zu halten und dadurch die Neigung für Aufspleißen an den Enden dieses Geflechts auf ein Minimum zu bringen, wobei die Beschichtung gestattet, daß die Monofilamente sich gegeneinander an ihren Überkreuzungsstellen drehen bzw. verschwenken, so daß sie die Ausdehnungsmerkmale dieses Geflechtes beibehalten, und wobei diese Bildungsstufe das Beschichten von praktisch allen freiliegenden Oberflächen dieser Monofilamente mit diesem elastomeren Material in fließfähiger Form ohne Füllen der Öffnungen zwischen diesen Monofilamenten umfaßt.

8. Verfahren nach Anspruch 7, dadurch gekennzeichnet, daß das Material aus der Gruppe gewählt ist, die aus Recorcin/Formaldehyd und Acryllatex besteht.

9. Verfahren nach Anspruch 7 oder 8, dadurch gekennzeichnet, daß die Beschichtung etwa 0,025 mm bis etwa 0,5 mm (etwa 1 bis etwa 20 mils) Dicke hat.

10. Verfahren nach irgendeinem der Ansprüche 7 bis 9, dadurch gekennzeichnet, daß die Bildung dieser Beschichtung das Durchführen dieses Geflechts durch ein Bad des elastomeren Materials in seiner fließfähigen Form umfaßt und danach das Verfestigenlassen dieses Matrials auf diesem Geflecht.

11. Verfahren nach Anspruch 10, dadurch gekennzeichnet, daß das elastomere Material in seiner fließfähigen Form eine Viskosität von nicht wesentlich größer als 15 N/s/m⁻² (15.000 cP) hat.

12. Verfahren nach irgendeinem der Ansprüche 7 bis 11, dadurch gekennzeichnet, daß man den festen Überzug über diesen Monofilamenten, und den Öffnungen zwischen ihnen bildet und danach dieses geflochtene Erzeugnis zusammendrückt, um diese Beschichtung in den Bereichen zu brechen, wo sie diese Öffnungen bedeckt.

## Revendications

1. Tresse à dilatation comprenant une pluralité de monofilaments tressés et un revêtement d'un matériau élastomère solide adhérent sur lesdits monofilaments, maintenant lesdits monofilaments dans leur position appropriée les uns par rapport aux autres pour empêcher l'évasement des extrémités de ladite tresse tout en permettant aux monofilaments de pivoter les uns par rapport aux autres à chacune de leurs jonctions afin de conserver les caractéristiques de dilatation de ladite tresse, les ouvertures entre lesdits monofilaments étant sensiblement exemptes dudit revêtement.

2. Tresse à dilatation selon la revendication 1, dans laquelle ledit matériau élastomère est sélectionné parmi le groupe consistant en résorcinol-formaldéhyde et latex acrylique.

3. Tresse à dilatation selon la revendication 1 ou 2, dans laquelle lesdits monofilaments sont en une matière plastique technique.

4. Tresse à dilatation selon la revendication 3, dans laquelle lesdits monofilaments sont en Nylon ou en polyester.

5. Tresse à dilatation selon l'une quelconque des revendications 1 à 4, dans laquelle ledit revêtement s'étend sur pratiquement toutes les surfaces exposées desdits monofilaments sur toute la longueur de ladite tresse.

6. Tresse à dilatation selon l'une quelconque des revendications précédentes, dans laquelle ledit revêtement a une épaisseur comprise entre 0,025 mm (1 millième de pouce) et 0,5 mm (20 millièmes de pouce).

7. Procédé de traitement d'une tresse à dilatation comprenant une pluralité de monofilaments tressés pour réduire sa tendance à s'évaser à ses extrémités tout en conservant ses propriétés de dilatation, caractérisé par la phase consistant à former un revêtement solide d'un matériau élastomère solide adhérent sur lesdits monofilaments de ladite tresse afin de les maintenir dans leur position appropriée les uns par rapport aux autres et donc de minimiser la tendance à l'évasement aux extrémités de ladite tresse, ledit revêtement permettant auxdits monofilaments de pivoter les uns par rapport aux autres à leurs jonctions afin de conserver les caractéristiques de dilatation de ladite tresse, ladite phase de formation du revêtement consistant à recouvrir pratiquement toutes les surfaces exposées desdits monofilaments avec ledit revêtement élastomère sous forme fluide sans remplir les ouvertures entre lesdits monofilaments.

8. Procédé selon la revendication 7, dans lequel ledit matériau est sélectionné parmi le groupe consistant en résorcinol-formaldéhyde et latex acrylique.

9. Procédé selon la revendication 7 ou 8, dans lequel ledit revêtement a une épaisseur comprise entre 0,025 mm (1 millième de pouce) et 0,5 mm (20 millièmes de pouce).

10. Procédé selon l'une quelconque des revendications 7 à 9, dans lequel ladite formation dudit revêtement comprend la phase consistant à passer ladite tresse dans un bain du matériau élastomère sous sa forme fluide, puis à laisser ledit matériau se solidifier sur ladite tresse.

11. Procédé selon la revendication 10, dans lequel ledit matériau élastomère sous sa forme fluide a une viscosité n'excédant pas 1 5 N/s/m⁻² ( 1 5 000 centipoises).

12. Procédé selon l'une quelconque des revendications 7 à 11, comprenant la phase consistant à former ledit revêtement solide sur lesdits monofilaments et les ouvertures entre eux, puis à comprimer ledit produit tressé afin de rompre ledit revêtement dans les régions où il recouvre lesdites ouvertures.
